

Dec. 20, 1938.

C. H. MAHONEY

2,140,534

ELECTRODE FOR ELECTRON DISCHARGE DEVICES

Filed Jan. 11, 1937

FIG. 2.



FIG. 1.



FIG. 3.



Inventor  
CHARLES H. MAHONEY.

by Charles Mahoney Atty.

## UNITED STATES PATENT OFFICE

2,140,534

ELECTRODE FOR ELECTRON DISCHARGE  
DEVICES

Charles H. Mahoney, Owensboro, Ky., assignor to  
The Ken-Rad Tube and Lamp Corporation,  
Owensboro, Ky., a corporation of Kentucky

Application January 11, 1937, Serial No. 119,928

2 Claims. (Cl. 250—27.5)

This invention relates to electrodes for electron discharge devices, and more particularly to magnetically shielded electrodes constructed in a novel manner and including an improved alloy having a high magnetic permeability at high temperatures.

With the advent of indirectly heated cathodes and the use of alternating current electricity as a source of heat for raising the temperature of a cathode to its desired electron emission point, a new problem presented itself to the radio engineer. It was found that the current flowing through the heating element set up an electro-magnetic field which reached out into the region of normal electron flow. This electro-magnetic field thus influenced the electrons emanating from the cathodes and thereby caused undesirable fluctuations of current in the anode circuit of the discharge device. Many suggestions have been proposed to overcome the effect of this electro-magnetic field, such for example, as by employing a heating element having a resistance wire which is wound in a reverse helical manner, the assumption being that the oppositely directed magnetic fields developed by the neighboring sections of a heating wire would cancel each other.

It has been found, however, that the more effective way of eliminating the undesirable effects of this magnetic field is to construct the cathodes with an inner shield composed of a material having a high magnetic permeability at high temperatures which will substantially prevent the electro-magnetic field referred to above from extending beyond the shield.

Thus it is an object of this invention to provide a novel shielded electrode construction.

It is a further object of this invention to provide an electrode having a shielding layer of novel composition.

It is a still further object of this invention to provide a cathode having a layer of ferrous-cobalt alloy, the cobalt content being sufficient to provide a stable magnetic transformation characteristic.

It is a still further object of this invention to provide a cathode having a layer of ferrous-cobalt alloy, the cobalt content being at least 19%.

Now in the construction of duo-metal articles, it is, of course, easier to manufacture them in sheets or strips and then form the desired article thereafter. Tubing composed of metal such as alloys having a ferrous-cobalt composition, however, cannot be readily welded, and tubing which has been formed with a locked seam or the like is objectionable in that it presents an irregular

surface for the coating of the electron emissive substance. Those skilled in the art will readily appreciate that an irregular coating of the electron emissive substance is readily chipped, thereafter rendering the discharge device unsatisfactory. It is thus an object of this invention to provide a novel seamless tube cathode construction for electron discharge devices.

It is a further object of this invention to provide a novel seamless tube cathode having a 10 layer of ferrous-cobalt alloy and a superimposed layer of some other metal.

Another and further object of this invention is to provide a novel cathode construction including a seamless tube of ferrous-cobalt alloy and a 15 second tube of non-ferrous metal disposed over the alloy tube, there being a welded bond therebetween.

Another and further object of this invention is to provide a novel cathode construction including 20 a tube of ferrous-cobalt-nickel alloy.

The novel features which I believe to be characteristic of my invention are set forth with particularity in the appended claims. My invention itself, however, both as to its composition and 25 manner of construction, together with further objects and advantages thereof, may best be understood by reference to the following description taken in connection with the accompanying drawing in which:

Figure 1 is an elevational view partly in cross-section, but not drawn to scale for purposes of clarity, of an electron discharge device;

Figure 2 is a cross-sectional end view of the cathode of the electron discharge device illustrated in Figure 1; and

Figure 3 is a diagram illustrating the magnetic transformation characteristic of the shielding material employed in the construction of the cathode illustrated in Figures 1 and 2.

In Figure 1 of the drawing, an electron discharge device 10 is illustrated and includes a cathode heating coil 11, a cylindrical cathode 12, a grid electrode 13, and a plate electrode or anode 14. Although discharge device of Fig. 1 is shown 45 as being provided with a single grid electrode, it is to be understood that the device may be provided with any number of grid electrodes or without any grid electrodes without departing from the spirit and scope of this invention.

Now the particular construction of cathode 12 (see Figures 1 and 2) constitutes one of the cardinal features of the present invention, and includes an inner layer 15 composed of a novel ferrous-cobalt alloy having a high magnetic permeability 55

characteristic at high temperatures. As will be presently pointed out this layer 15 prevents the electro-magnetic field set up by the flow of current through heating coil 11 from extending into the region of normal electron flow which exists in the space 16 between cathode 12 and anode 14. As is the common practice in the construction of electron discharge devices of the indirectly heated cathode type, cathode 12 includes an outer layer 17 of some suitable electron emissive substance, such as an oxide of the alkaline earth group. In order to prevent any chemical reaction between layer 17 and the ferrous-cobalt alloy layer 15, a layer 18 of non-ferrous metal such as nickel or copper is interposed between the electron emissive substance 17 and the ferrous cobalt alloy 15. Preferably, this metal should be a good conductor of electricity, non-reactive chemically to the electron emissive substance, and have good adhesion properties with respect to the electron emissive substance.

It has been found that when inner layer 15 of cathode 12 is constructed from a ferrous-cobalt alloy having a certain predetermined minimum percentage of cobalt therein, a very effective magnetic shield is obtained. In Figure 3 of the drawing, the magnetic transformation curve M of ferrous-cobalt alloys is illustrated. The percentage of cobalt in the alloy is plotted as the abscissae of the curve while the temperatures at which the Curie point or magnetic transformation takes place is plotted as the ordinates of the curve. Upon inspection of Figure 3 of the drawing, it will be noted that the left hand portion of the curve M is divided into two portions M<sub>1</sub> and M<sub>2</sub>. The region B between zero percentage of cobalt and approximately 21% cobalt constitutes an unstable transformation region. Since the usual maximum temperature at which the cathode of an electron discharge device operates is approximately 900°, it has been found important to have a cobalt content in the alloy sufficient to cause operation along or near the stable portion of the magnetic transformation curve M. That is to say, it is desirable to have at least 19% cobalt content in the alloy.

Since additional cobalt may result in intricate metallurgical practice being necessary, and since it is desirable to have the alloy as malleable as possible to permit ready working of the metal, the cobalt content is preferably only slightly greater than 21%.

One extremely satisfactory method of forming a ferrous cobalt alloy such as that described above into a seamless tube cathode structure 12 is to first hot or cold draw a tube of ferrous cobalt alloy to within two or three of the final passes, and then electroplate a metal such as nickel thereon. The plated tubing is then redrawn to effect a welded bond between the ferrous-cobalt alloy and the nickel plating. After this hot or cold working operation, the tubing is again electroplated with nickel and then redrawn until the desired tube size and coating thickness are obtained. Thereafter, a coating of an electron emissive substance such as one of the oxides of the alkaline earth group may be applied to the outer surface of the nickel in the conventional manner. This bonding of the plated tubing substantially eliminates blistering of the nickel on the alloy.

A second satisfactory method of constructing a

seamless tube cathode having an inner layer of ferrous-cobalt alloy includes hot or cold drawing a tube of ferrous-cobalt alloy to approximately its desired final size. A pre-drawn tube of nickel having an inside diameter substantially the same as the outside diameter of the drawn ferrous-cobalt alloy tube is then slipped or forced over the latter. This assembly is then hot or cold drawn to size to effect a welded bond between the two metals. Thereafter a coating of an electron emissive substance such as one of the oxides of the alkaline earth group is applied to the outer surface of the nickel in the conventional manner.

Although the relative dimensions of the respective layers of the cathode may vary through wide ranges without departing from the spirit and scope of this invention, the only purpose of the nickel layer is to function as a chemical shield between the ferrous-cobalt alloy and the emissive coating. Now the magnetic shielding effect of the ferrous cobalt alloy increases with the wall thickness. Therefore, it is desirable that the nickel wall be made as thin as is commensurate with the obtaining of a continuous chemical shield so that as much of the total wall thickness as is possible will be available for the magnetic shielding alloy. It is desirable to keep the combined cathode wall thickness as thin as possible for the following reasons:

1. For ease of degasification of material.
2. To facilitate quick heating.
3. As space conservation for heater.

(Usually in practice it ranges from .001" to .005".)

Although I have described nickel as being electrolytically deposited on a ferrous cobalt alloy, it is to be understood that the process may be reversed and the ferrous cobalt alloy electrolytically deposited on the nickel without departing from the spirit and scope of this invention.

While I have described particular embodiments of my invention, it will, of course, be understood that I do not wish to be limited thereto, since many modifications may be made, and I therefore contemplate by the appended claims to cover all such modifications as fall within the true spirit and scope of my invention.

I claim as my invention:

1. A laminated cathode for electron discharge devices comprising an inner layer of magnetic shielding material composed of a malleable ferrous-cobalt alloy having a cobalt content of at least 19% and a ferrous content of approximately 75% to 80%, an outer layer of an electron-emissive surface, and an intermediate layer of a non-ferrous metal of good electrical conductivity to prevent chemical reaction between said outer layer and said inner layer, said intermediate layer being intimately bonded to said inner layer as in the drawing of a laminated tube composed of said inner and intermediate layers.

2. A malleable laminated cathode for electron discharge devices comprising a layer of ferrous-cobalt alloy composed of at least 19% cobalt and a ferrous content of approximately 75% to 80%, intimately bonded to a layer of a non-magnetic material of high electrical conductivity, said layer of high conductivity being adapted to receive a layer of an electron emissive surface.